

1,197,705.

R. WINNE.  
INCANDESCENT ELECTRIC LAMP.  
APPLICATION FILED APR. 24, 1913.

Patented Sept. 12, 1916.



Witnesses:

*George H. Tilden*  
*J. Ellis Kler.*

Inventor:

Roy Winne,  
by *Albert S. Davis*  
His Attorney.

# UNITED STATES PATENT OFFICE.

ROY WINNE, OF SCHENECTADY, NEW YORK, ASSIGNOR TO GENERAL ELECTRIC COMPANY, A CORPORATION OF NEW YORK.

## INCANDESCENT ELECTRIC LAMP.

1,197,705.

Specification of Letters Patent. Patented Sept. 12, 1916.

Application filed April 24, 1913. Serial No. 763,263.

To all whom it may concern:

Be it known that I, ROY WINNE, a citizen of the United States, residing at Schenectady, in the county of Schenectady, State 5 of New York, have invented certain new and useful Improvements in Incandescent Electric Lamps, of which the following is a specification.

The present invention relates to incandescent lamps, and especially to lamps provided with a metal filament, particularly a tungsten filament.

It is one of the objects of my invention to increase the useful life of such lamps and 15 also to maintain the efficiency at which the filament is operating substantially constant at a high value.

When a tungsten filament is operated in an evacuated bulb under ordinary conditions, the resistance of the filament gradually increases, thus lowering its temperature, and the bulb is progressively darkened by a black deposit of vaporized tungsten. Both these effects contribute to lowering the 25 efficiency and candle power of the lamp. When the efficiency has been reduced to a certain value, say 80%, the lamp has reached the end of its useful life.

In order to increase the length of life of 30 a lamp at a given efficiency various solid halogenous compounds of low vapor tension, such as potassium thallium chlorid, cryolite, or potassium iodid have been placed in the lamp. These compounds are placed 35 in the lamp in such a position that when the filament is at normal incandescence and the bulb is well evacuated there is evolved an atmosphere which is chemically active to the metal of the filament and which is of sub- 40 stantially the pressure of a first class vacuum, as lamps in which the compounds are properly placed respond to vacuum tests in the same way as lamps which have a first class vacuum.

45 I have discovered that the useful life of a lamp may be still more increased by placing in the bulb with a regenerative compound of this nature a very small amount of gas, preferably nitrogen.

.50 The accompanying drawing shows one form of incandescent lamp to which my invention may be applied.

In carrying my invention into effect the bulb 1 is first provided with the filament 2,

mounted upon a support 3 and is connected 55 to leading-in conductors 4, 5, which are sealed into the stem 6 and connected as usual to the base contacts 7 and 8. The lamp is provided with a small amount of compound 9 which in the case of potassium thallium 60 chlorid is contained in a small open tube 10. As indicated the salt is held in place by glass wool 11. The tip of the tube may be contracted as indicated at 12.

The bulb is exhausted on the rough pump 65 and finally heated for about 12 minutes at 340°-360° C. while completing the exhaustion on the fine pump. The temperature is then lowered to about 250°-270° C. and about 50% of the normal lamp voltage is im- 70 pressed upon the filament. The lamp is run in this way until the vacuum becomes as good as about 2 microns. The heating and current are then discontinued and about 100 microns of dry nitrogen admitted. The fila- 75 ment is incandesced for about 10 seconds and the gas pumped out again to about 2 microns' pressure. More dry nitrogen to the desired pressure is admitted and the bulb is then sealed off. Ordinarily the pres- 80 sure of the gaseous atmosphere should be less than 100 microns, and usually within the range of about 10 to 50 microns, or .010 to .050 millimeter of mercury. A gas pres- 85 sure as great as 100 microns is apt to pro- duce destructive electrical discharges be- 90 tween the leads at commercial voltages, such as 110 volts or higher. Of course, this par- ticular procedure may be varied considera- bly in accordance with the character of the lamp and other conditions.

To illustrate the effect of my novel filling combination on the life of the lamp, I desire briefly to cite several specific examples. A 125 volt, 100 watt lamp, having a drawn 95 tungsten filament was provided with a small amount of potassium thallium chlorid placed in the same way as in a vacuum lamp. The bulb was evacuated as above described and then enough dry nitrogen gas was admitted 100 to produce an atmosphere of about 25 mi- crons (0.025 mm. of mercury) pressure. The lamp was then sealed off and operated at an efficiency of .95 watt per candle. After 1900 hours the candle power had fallen 105 only to 96% of its original value. During the operation of the lamp the resistance of the filament repeatedly increased several

per cent. and then came back to normal. In the absence of the nitrogen the efficiency of a lamp of this type containing potassium thallium chlorid would have fallen to about 5 80% in about 1000-1200 hours. A similar lamp provided in the same manner with potassium thallium chlorid and nitrogen was found after operating 1000 hours at .95 watt per candle to have actually increased 10 in efficiency, as it was operating at 101% of its original candle power.

While I prefer to use nitrogen gas, I find that a small amount of air, carbon dioxid, oxygen, and even hydrogen may be similarly 15 used although with less beneficial effect in the order mentioned.

While the benefits of my invention may be secured irrespective of any theory, it may be said that the following reactions perhaps 20 take place. When nitrogen is used, for example, tungsten vaporized by the incandescence of the filament is probably converted into tungsten nitrid. This would soon exhaust the supply of nitrogen but the nitrid 25 is decomposed by the halogen compound to regenerate nitrogen. The tungsten compound on its part is decomposed at the temperature of the filament, depositing tungsten on the surface of the filament. I do 30 not wish to be limited, however, by this theory of the behavior of the lamp.

What I claim as new and desire to secure by Letters Patent of the United States, is:—

1. An incandescent lamp comprising an 35 envelop, a metal filament therein, a solid halogenous compound placed therein to evolve when said filament is at normal incandescence in a first class vacuum a vapor chemically active to the material of the filament and at substantially the pressure of a 40 first class vacuum, and a charge of gas hav-

ing an initial pressure less than one tenth of a millimeter of mercury.

2. In an incandescent lamp, the combination with an envelop having a tungsten filament therein, and potassium thallium chlorid placed in said envelop to evolve in the evacuated envelop at normal incandescence of the filament an atmosphere of vapor at substantially the pressure of a first class 50 vacuum, of nitrogen gas in said envelop at a pressure of about .010-.050 millimeter of mercury pressure.

3. An incandescent lamp comprising an envelop containing a tungsten filament, a solid halogenous compound which evolves at normal incandescence of the filament when said envelop is evacuated to a first class vacuum an atmosphere of vapor chemically active to tungsten and of a pressure 60 substantially that of a first class vacuum, and a charge of nitrogen having an initial pressure less than one tenth of a millimeter of mercury.

4. An incandescent lamp comprising an envelop containing a tungsten filament, a solid halogenous compound which evolves at normal incandescence of the filament when said envelop is highly evacuated an atmosphere chemically active to tungsten and of 70 a pressure substantially that of a first class vacuum, and a charge of nitrogen having an initial pressure higher than that of a first class vacuum and lower than that which permits electrical discharge in the bulb at 75 normal voltage.

In witness whereof, I have hereunto set my hand this 23rd day of April, 1913.

ROY WINNE.

Witnesses:

BENJAMIN B. HULL,  
HELEN ORFORD.